

Sept. 10, 1929.

K. V. McCausland

1,727,514

ART OF TEEMING FERROUS METALS

Filed Nov. 8, 1927

*Fig. 1.*



*Fig. 2.*



884

Inventor

*Karl V. McCausland*

*Hoppe and Rivers.*

Attorney

## UNITED STATES PATENT OFFICE.

KARL V. McCausland, OF BUFFALO, NEW YORK.

## ART OF TEEMING FERROUS METALS.

Application filed November 8, 1927. Serial No. 231,918.

This invention relates to the art of teeming ferrous metals and involves improvements in the method of and means for preparing the teeming ladle for the teeming operation, whereby to secure the free flow of the metal, and the easy release and accurate seating of the stopper.

An object of the invention is to prevent the formation of skull, or freezing of metal, in the immediate vicinity of the teeming ladle nozzle, thereby to insure the free opening and tight closing of the nozzle during the teeming operation.

Another object of the invention is to position a deoxidizing substance within the teeming ladle in a manner such that it is useful for the dual purpose of preventing skull and deoxidizing.

A further object of the invention is to provide the substance in a form and relation such that it will be retained in position during its action.

In connection with the casting of ingots, the usual practice is to run the molten metal into the ladle and then teem it from the bottom of the ladle to the ingot mold. It is well established in such practice that the best results are obtained when the temperature of the metal is as low as possible consistent with a free running condition. With this in mind, it will be readily appreciated that when the metal is tapped into the ladle, the first mass of metal coming into contact with the comparatively cold surface of the ladle bottom is very apt to be chilled sufficiently to reduce its temperature to the freezing point and thus form a skull around the teeming nozzle and the end of the stopper. Such formation seriously interferes with the proper manipulation of the stopper, and quite often prevents the end of the stopper from seating tightly into nozzle orifice so that the flow of metal cannot be shut off. This condition is highly objectionable inasmuch as it obviously prevents clean casting, increases scrap and is extremely dangerous to the workers.

I have discovered that the skull formation in the immediate vicinity of the nozzle may be eliminated, together with its attendant objections, by securing a substance

or element around the nozzle, prior to the tapping operation, which will be quickly melted by the molten metal when it is tapped into the ladle. The substance to which I refer, may be aluminum, magnesium, an alloy thereof, or any other equivalent substance having a comparatively low melting point and which, upon melting, will react with the oxygen in the metal to generate heat.

An embodiment of my invention is illustrated in the accompanying drawings wherein:

Figure 1 is a vertical cross sectional view of the ladle with the substance in position around the nozzle of the stopper.

Figure 2 is a perspective view of the ring.

In order to practice my invention, I utilize the usual type of teeming ladle as indicated at 1, having a nozzle 2, a stopper 3, and an actuating handle 4, by means of which the stopper is raised and lowered to open or close the nozzle. Before tapping any metal into the ladle, the aluminum or other substance 5 is placed adjacent the nozzle and securely held there so that it will not float upwardly upon the surface of the metal when the latter is tapped. In the preferred embodiment of my invention, I construct the element 5 in the form of a ring which may be placed around the end of the stopper 3, the diameter of the ring being large enough to fit over the stopper but small enough to prevent it from rising upwardly along the stopper.

Obviously as the molten metal is tapped into the ladle it will completely cover the ring. Due to the comparatively low melting point of the ring and the comparatively high temperature of the metal, the ring will be melted in a very short space of time. The fluid aluminum thus produced will mix with the surrounding metal, and the resulting mixture will have a freezing point lower than that of the metal alone. Hence, by lowering its freezing point in this manner, it is caused to remain in a free running condition. This condition is further insured by the reaction between the aluminum and the oxygen of the metal, inasmuch as such reaction generates heat and thereby actually causes a rise

in the temperature of the metal. The two actions mentioned here are not necessarily consequent upon one another, and it will, therefore, be seen that I can use one substance as a deoxidizer and another to prevent skull, but naturally I prefer a substance that performs both functions. While the complete action which takes place does so in a comparatively short time, I have found that it effectually prevents any initial skull formation.

The insertion of aluminum into teeming ladles for the purpose of deoxidizing the molten metal which is contained or tapped therein, is, of course, well known in this art. In such practice however, no attempt heretofore, has been made to retain the aluminum near the nozzle while it melted. As a result it has always floated on the surface of the metal, and its melting had little or no effect upon the skull formation at the bottom of the ladle. Obviously, however, my ring will form a part of the weight of aluminum usually added for deoxidizing purposes and, therefore, will fulfill the dual purpose of deoxidizing and preventing freezing as before related.

From the foregoing description, it will be apparent that I have devised a particularly simple and also an efficient means for preventing the freezing of metal around the stoppers of teeming ladles and one which can be used upon any standard type of ladle without necessitating the alteration of its construction or adding materially to the cost of manufacture either through extra labor or materials. Although I have illustrated and described a preferred embodiment of my invention, it is to be understood that I can substitute any other equivalent substance in place of aluminum or magnesium. It is also to be understood that various changes in the construction of my particular substance and the retaining means therefore can be made without departing from the spirit of my invention or the scope of the appended claims.

I claim as my invention:

1. In the art of teeming metal a method of preparing a teeming ladle having a stopper controlled discharge nozzle for the teeming operation consisting in placing a metallic reducing substance having a comparatively low melting point in the vicinity of the nozzle prior to tapping the metal to be teemed, into the ladle.

2. In the art of teeming ferrous metals, a method of preparing a teeming ladle having a stopper controlled discharge nozzle for the teeming operation consisting in placing a metallic reducing substance having a comparatively low melting point in the vicinity of the nozzle prior to tapping the ferrous metal into the ladle, and relatively

maintaining the position of the substance until melted by said metal.

3. In the art of teeming ferrous metals, a method of preparing a teeming ladle having a stopper controlled discharge nozzle for the teeming operation consisting in placing a metallic deoxidizing substance having a comparatively low melting point in the vicinity of the nozzle prior to tapping the ferrous metal into the ladle.

4. In the art of teeming ferrous metals, a method of preparing a teeming ladle having a stopper controlled discharge nozzle for the teeming operation consisting in placing a body of aluminum around the nozzle end of the stopper prior to tapping the ferrous metal into the ladle.

5. In the art of teeming ferrous metals, a method of preparing a teeming ladle having a stopper controlled discharge nozzle for the teeming operation consisting in placing a body of aluminum around the nozzle end of the stopper prior to tapping the ferrous metal into the ladle, and relatively maintaining the position of said body until melted by said metal.

6. In the art of teeming ferrous metals, a method of preparing a teeming ladle having a stopper controlled discharge nozzle for the teeming operation consisting in placing a ring of aluminum around the nozzle end of the stopper prior to tapping the ferrous metal into the ladle, the internal diameter of said ring being small enough to prevent it from rising upwardly along the stopper.

7. Teeming apparatus comprising a ladle having a nozzle, a stopper for said nozzle, and a ring placed on the nozzle end of said stopper, said ring being composed of a metallic reducing substance having a comparatively low melting point with respect to the metal to be teemed.

8. Teeming apparatus comprising a ladle having a stopper controlled nozzle and a ring fitted on the nozzle end of said stopper, said ring being composed of a metallic deoxidizing substance having a comparatively low melting point with respect to the metal to be teemed.

9. A method of teeming metal consisting in placing and maintaining adjacent the stopping controlled teeming opening, a metallic reducing substance having a melting point lower than that of the metal to be teemed and thereafter tapping and teeming the metal.

In testimony whereof I affix my signature.

KARL V. McCausland.